

## UNITED STATES PATENT OFFICE

ALWIN MITTASCH, AND CARL MÜLLER, OF MANNHEIM, AND EDUARD LINCKH, OF LUDWIGSHAFEN-ON-THE-RHINE, GERMANY, ASSIGNORS TO I. G. FARBENINDUSTRIE AKTIENGESELLSCHAFT, OF FRANKFORT-ON-THE-MAIN, GERMANY, A CORPORATION OF GERMANY

## PRODUCTION OF PURE IRON

No Drawing. Application filed July 2, 1927, Serial No. 203,258, and in Germany July 5, 1926.

It is known that pure iron can be produced from iron carbonyl by thermal decomposition by passing the iron carbonyl, in a vaporous and diluted condition, that is in the presence of inert or reducing gases or under diminished pressure, through heated liquids or melts.

We have now found that it is not essential to employ the iron carbonyl in a diluted condition, but that it is often preferable to bring it in an undiluted liquid or vaporous condition into contact with the hot liquid or melt. If, for example, the decomposition be effected by introducing iron carbonyl into molten iron, the method according to the present invention is preferable to employing a gas which dilutes the carbonyl vapor, since such gas extracts considerable quantities of heat in its passage through the melt.

20 The decomposition of the iron carbonyl can be carried out for example by passing the liquid or vaporous carbonyl through the heated liquid or melt at ordinary or under increased pressure, or by bringing it, in the form of vapor, into contact with the surface of a suitably agitated liquid or melt, or by spraying or dropping it, in the liquid condition, onto the liquid.

The working temperatures generally employed are between 100° and 400° C or above 1000° C. in order to prevent extensive deposition of carbon as the result of the decomposition of carbon monoxid at the intermediate range of temperature. If, however, it is desired to obtain an iron possessing a certain high content of carbon or iron carbide, the decomposition is effected at temperatures between 400° and 1000° C.

Organic liquids of high boiling point, such as paraffin oils and the like, have been found suitable substances for the decomposition process. Substances of lower boiling point may also be used, provided the operation be carried out in closed vessels under pressure.

45 The decomposition may also be effected with the aid of melts of salts or metals, in which case, according to the nature of the melt, the resulting iron is deposited either in the form of a fine powder, as when heated liquids are used, or is dissolved in the melt as, for ex-

ample, when the decomposition is effected in molten iron, the metal being then produced directly in a pure, compact state.

The process according to the present invention has the advantage that no gas is required for diluting the carbonyl, for which purpose no industrial gas can generally be employed, as such diluting gas must be dry and free from oxidizing constituents, so that it is rather expensive to produce. Moreover, by the absence of a diluting gas a considerably smaller supply of heat is necessary, as no gas must be heated together with the carbonyl. Further, in the present process pure carbon monoxid is recovered while in the operation with diluted iron carbonyl the carbon monoxid is strongly diluted with other gases and therefore not suitable for all industrial purposes, unless pure carbon monoxid itself be employed as diluting gas.

70 The following example will further illustrate how the invention may be carried out in practice, but the invention is not restricted thereto.

## Example

Liquid iron carbonyl is allowed to drop gradually into a colorless paraffin oil, heated to 270° C. The resulting iron remains suspended, as a fine powder, in the oil. The bulk of the oil can be separated from the iron by centrifuging, and washing with ether furnishes a very pure and finely divided iron powder of uniform grain size.

## What we claim is:

75 The process of producing pure iron which comprises bringing undiluted iron carbonyl in contact with fused iron.

In testimony whereof we have hereunto set our hands.

ALWIN MITTASCH.  
CARL MÜLLER.  
EDUARD. LINCKH.

90

95

100